

April 24, 1973

TAKAHO KAWAWA

3,729,309

METHOD FOR ADDING ALLOYING ELEMENTS TO MOLTEN METALS

Filed March 2, 1970

5 Sheets-Sheet 1

FIG. 1



INVENTOR  
TAKAHO KAWAWA  
BY *Steinberg & Blake*  
ATTORNEYS

April 24, 1973

TAKAHO KAWAWA

3,729,309

METHOD FOR ADDING ALLOYING ELEMENTS TO MOLTEN METALS

Filed March 2, 1970

5 Sheets-Sheet 2

FIG. 2



FIG. 3



INVENTOR  
TAKAHO KAWAWA  
BY *Steinberg & Blake*  
ATTORNEYS

April 24, 1973

TAKAHO KAWAWA

3,729,309

METHOD FOR ADDING ALLOYING ELEMENTS TO MOLTEN METALS

Filed March 2, 1970

5 Sheets-Sheet 3

FIG. 4



FIG. 5



INVENTOR  
TAKAHO KAWAWA  
BY  
Steinberg + Blake  
ATTORNEYS

April 24, 1973

TAKAHO KAWAWA

3,729,309

METHOD FOR ADDING ALLOYING ELEMENTS TO MOLTEN METALS

Filed March 2, 1970

5 Sheets-Sheet 4

FIG. 6



FIG. 7



INVENTOR  
TAKAHO KAWAWA  
BY *Steinberg + Blake*  
ATTORNEYS

April 24, 1973

TAKAHO KAWAWA

3,729,309

METHOD FOR ADDING ALLOYING ELEMENTS TO MOLTEN METALS

Filed March 2, 1970

5 Sheets-Sheet 5

FIG. 8



INVENTOR  
TAKAHO KAWAWA  
BY *Steinberg + Blake*  
ATTORNEYS

## 1

3,729,309

METHOD FOR ADDING ALLOYING ELEMENTS  
TO MOLTEN METALSTakaho Kawawa, Kawasaki, Japan, assignor to Nippon  
Kokan Kabushiki Kaisha, Tokyo, Japan  
Filed Mar. 2, 1970, Ser. No. 15,339

Claims priority, application Japan, Feb. 7, 1969,

44/17,041

Int. Cl. C22c 1/06, 33/00

U.S. CL. 75—129

7 Claims

## ABSTRACT OF THE DISCLOSURE

A method for adding alloying elements such as aluminum, titanium to molten metals, said elements being capable of reacting with the atmosphere surrounding the metals, comprising inserting a wire rod made of the element into a molten metal bath at a controlled speed, said rod having a controlled size, so as to produce a refined and purified metal alloy.

This invention relates to a method for adding alloying elements to molten metals during a refining procedure. More particularly, it relates to the addition of such elements which are liable to be converted into either a nitride or oxide by reaction with the atmosphere ambient to the molten metals in a container such as a ladle.

The said alloying elements, i.e., Si, Al, Ti, V, La, Nb, or alloys containing one or more of the above have been added in the form of a lump, a bar or the like to molten steel by conventional methods, wherein they are either added directly to the molten metals tapped into a ladle or placed in a ladle prior to the teeming. By these conventional methods, the yield of Al and Ti is low and unstable because of the ready reaction thereof with the atmosphere, although various shapes of Al and Ti have been proposed in order to promote a high yield in steelmaking.

The low and unstable yield of Al and Ti results from an oxidation loss caused by their reaction with either oxygen or oxidizing slag in the molten steel or the atmosphere surrounding the molten steel during tapping. The dimensions of the atmosphere involved during tapping is 20 to 30 times larger than that of the molten steel, thus leading to a large oxidation loss. In the case of Ti and Ti alloy, the oxidation loss is increased by a reaction with nitrogen in the atmosphere.

For the above discussed reasons, it is expensive to produce a steel alloy containing elements with a high oxidizing or nitriding capacity, such as Ti and Al, by conventional methods. Moreover, Al, Ti and their alloys react with the atmosphere to form a great amount of  $Al_2O_3$ ,  $TiO_2$  and  $TiN$ . The amount of the respective alloying elements is unstable in the molten steel, which decreases the quality of the steel alloys.

This invention relates to a method of adding alloying elements, liable to react with the atmosphere, to the initially refined molten metals. In the method of the invention Al, Ti and alloys containing the same are added to the molten steel in the form of a wire rod at a speed ranging from 2.5 to 50 m./sec. while the steel is stirred.

For a better understanding of the invention reference will now be made to the accompanying drawings in which:

FIG. 1 illustrates an apparatus embodying the present invention;

## 2

FIGS. 2 to 4 are cross-sectional views of different stirring devices;

FIG. 5 is a graph showing the deviation of Sol. Al in a steel alloy using a conventional method;

FIG. 6 is a graph showing deviation of Sol. Al in a steel alloy using a method embodying this invention;

FIG. 7 is a graph showing deviation of Ti in a steel alloy obtained by a conventional method; and

FIG. 8 is a graph showing deviation of Ti in a steel alloy obtained by a method embodying the present invention.

Referring now to FIG. 1, the primary refining procedure is completed in a furnace 1, wherein the necessary alloying elements are added prior to the addition of the elements, liable to be transformed into nitride or oxide, in such a way as to improve the yield of the latter elements. Said primarily refined molten metals are transferred from the furnace to a ladle 2, having a porous refractory material 3 forming part of its surface. Through the refractory materials gases which are harmless to the steels, such as Ar and  $N_2$ , are blown. The alloying agents in the shape of wire are fed through a reel 4 and guides 5 and 6 by means of a wire feed device 7 and inserted into the molten steel or iron at high speed.

It should be noted that the diameter of said wire rod ranges from 3 to 20 mm. and the adding speed ranges from 2.5 to 50 m./sec. A wire rod of less than 3 mm. in diameter is apt to be entangled in the guide 7 and cannot be fed with ease, whereas one of more than 20 mm. in diameter cannot be bent along the guide 7 with ease. Alloying agents with a lower specific gravity than iron, especially Al and Ti, will float on to the molten steel surface and will not disperse throughout the steel if added at a speed of less than 2.5 m./sec. If added at a speed of more than 50 m./sec., said alloying agents are concentrated at the point where the wire rod is inserted, and the extra alloy material floats on to the molten metal surface, thus impeding uniform distribution of the additive elements. Accordingly, the adding speed has to be controlled so as to promote uniform distribution of the alloy compositions.

In order to stir the molten steel in the ladle, various kinds of gas blowing devices are employed, e.g. a stopper type and a rotatable stopper type. The first type of ladle is provided with a porous refractory material 8 inside thereof as shown in FIG. 2 and the latter type of ladle is provided with the porous refractory material 8 at the end of the rotatable stopper as shown in FIG. 3. FIG. 4 shows an electric stirring system by means of a coil 10 supplying induction power to steel positioned in the ladle. In short, any stirring method for uniformly stirring the whole molten steel in the ladle is applicable for the uniform dispersion of said alloying agents and oxidizing agents added at a high speed in the molten bath. A stirring system of this kind not only helps in the uniform dispersion of the alloy agents in the bath but also makes such inclusions as  $Al_2O_3$ ,  $TiO_2$  and  $TiN$  formed by Al and Ti and their alloy additions float up to the surface, thus providing advantages in manufacturing refined and purified steel alloy.

In the method of the present invention, the alloying agents in the form of wire rod are directly dispersed throughout the molten steel without a reaction with slag or the atmosphere, thus improving the yield in steel making.

The invention is illustrated by the following examples.

**3**  
**EXAMPLE 1**

Fe-Mn, Fe-Si and Al have been conventionally added in the form of bars of 1 kg. weight at the tapping stage of manufacturing steel plates for shipbuilding in a top-blown converter of 100 ton weight. The deviation of said Sol. Al product by this method is shown in FIG. 5. On the contrary, the present invention provides a method in which only Fe-Mn and Fe-Si are added at the time of tapping and then Al wire rod of 10 mm. in diameter is added at a speed of 5-10 m./sec. over a period of five minutes after tapping while stirring the molten steel by argon or nitrogen gas blown by the device shown in FIG. 1. FIG. 6 shows the distribution of Sol. Al in a product so produced. A comparison of FIGS. 5 and 6 shows the yield point of Sol. Al is two times as high and the deviation is less by  $\frac{1}{2}$ . It should be noted that the desired or aimed value of Al content is easily obtained. The oxygen content of conventional steel alloy is  $T(O)=50\pm30$  p.p.m. while that of the steel alloy produced by the method of the invention is  $(T(O)=30\pm15$  p.p.m. Thus a good purified steel alloy is produced.

**EXAMPLE 2**

When AISI 321 steel produced in a 40 ton electric furnace is tapped into a ladle, bar-shaped Al and Fe-Ti alloy have been added simultaneously in the known method. By the present invention, the other alloying elements except Al and Ti are first added to a ladle in the conventional way and then Al wire rod of 8 mm. in diameter is inserted at a speed of 5 m./sec. and Ti wire rod of 10 mm. in diameter is inserted at the speed of 6 m./sec. successively. This steel requires 5 times as much Ti addition as compared with carbon steel. FIG. 7 shows deviation of Ti in the steel by the conventional method and FIG. 8 shows the result obtained by the present invention. These two figures clearly indicate that the yield point is 4 times higher, the standard deviation of alloying elements is  $\frac{1}{2}$  times less. The desired value of each alloying element can easily be obtained by the present invention as compared with the prior art.

It should be noted that the method of this invention decreases formation of TiN in the molten metals because of the high speed addition of Ti wire rod to a ladle and produces 0.4 mm. cold rolled steel plates of greatly improved yield ranging from 90 to 95% as a result. A large amount of TiN inclusion occurs in known method because of reaction with the atmosphere and therefore only 60 to 80% of the 0.4 mm. cold rolled steel plates were rated as first class. These data show the advantages of the present method for the manufacture of 0.4 mm. cold rolled steel plates.

**EXAMPLE 3**

When aluminium killed steel is manufactured from a 14 ton ingot with less than 0.06% of carbon content, 0.2 to 0.3% of manganese content and respectively less than 0.015% of phosphorus and sulphur content, the method of the invention provides for an improved and stable yield of Al as compared with the conventional method as shown in the following table. Clean steel alloy with little inclusions is produced by the present method.

**COMPARATIVE ANALYSIS OF MOLTEN METALS IN MOLDS [The mean value of 10 steel ingots]**

|                          | Al content (mean value) | Sol. Al percent (standard deviation) | Yield of Al, percent | Oxygen content, percent |
|--------------------------|-------------------------|--------------------------------------|----------------------|-------------------------|
| Conventional method      | 0.044                   | 0.010                                | 42                   | 0.0035                  |
| Present invention method | 0.045                   | 0.004                                | 63                   | 0.0025                  |

NOTE.—Yield of Al percent = (Sol. Al percent/added Al percent)  $\times 100$ .

**EXAMPLE 4**

Titanium killed steel, namely AISI steel 321, is produced from a 14 ton steel ingot with less than 0.08% 75

of carbon, 17.0 to 19.0% of chromium, 8.0 to 9.0% of nickel, less than 2% of manganese, less than 1% of silicon, less than 0.04% P, less than 0.03% of sulphur and 5 times more titanium than carbon. Such an alloying composition can be accurately obtained by the present invention because of the high yield of titanium, vanadium and the like as well as aluminium as is indicated in the table hereinbelow.

**COMPARATIVE ANALYSIS OF MOLTEN METALS IN MOLDS**

|                          | Ti content percent (mean value) | Standard deviation of Ti, percent | Yield of Ti, percent | Oxygen content, percent |
|--------------------------|---------------------------------|-----------------------------------|----------------------|-------------------------|
| Conventional method      | 0.41                            | 0.07                              | 23.1                 | 0.006                   |
| Present invention method | 0.39                            | 0.01                              | 91.2                 | 0.003                   |

**EXAMPLE 5**

The following table shows the comparative results in producing rimmed steels containing 0.05 to 0.06% of carbon, 0.30 to 0.50% of manganese and less than 0.020% of phosphorus and sulphur respectively.

**ANALYSIS OF OXYGEN CONTENT (PERCENT) IN MOLD AND FIRST CLASS YIELD OF COLD ROLLED STEEL**

|                          | Oxygen content (percent) $\pm$ standard deviation (percent) | First class yield of cold rolled steel plate, percent |
|--------------------------|-------------------------------------------------------------|-------------------------------------------------------|
| Conventional method      | 0.053 $\pm$ 0.006                                           | 85.5                                                  |
| Present invention method | 0.052 $\pm$ 0.003                                           | 89.4                                                  |

Accurate control of Sol. Al content means free control of the oxygen content of rimmed steel or semi-killed steel. Rapid analysis of the oxygen content of the molten metals prior to tapping facilitates manufacture of cold rolled steel plates of high quality both on the surface and internally with a much improved yield under the optimum rimming treatment based on the controlled oxygen content.

The method of the invention is applicable not only to Al and Ti but also to any other metallic alloying element, which is liable to react upon the atmospheric conditions, and which is capable of being formed into a wire rod.

I claim:

1. A method of uniformly alloying molten steel in a molten bath thereof with an alloying element, said element being capable of reaction with the atmosphere above said bath, which comprises continuously feeding a wire rod of said alloying element and having a diameter ranging from 3 to 20 mm. into said molten steel bath at a speed of 2.5 to 50 meters per second, while separately stirring the whole of said molten steel bath by a means non-reactive with said molten steel bath so that as said wire rod is consumed upon entering said molten steel bath said bath is being stirred, thereby uniformly distributing said alloying element therein, thus permitting formation of a steel alloy of uniform predetermined composition.

2. A method as claimed in claim 1, wherein the alloying element is titanium.

3. A method as claimed in claim 1, wherein the alloying element is aluminium.

4. A method as claimed in claim 1, wherein the alloying element is selected from the group consisting of silicon, vanadium, lanthanum and niobium.

5. A method as claimed in claim 1, wherein a plurality of wires are fed successively into the molten steel bath.

6. Method according to claim 1 wherein said molten steel bath is stirred by blowing inert gas therethrough.

7. Method according to claim 1 wherein said molten steel bath is stirred by subjecting said molten steel bath to electrical induction.

(References on following page)

## UNITED STATES PATENTS

|           |         |             |         |
|-----------|---------|-------------|---------|
| 2,253,574 | 8/1941  | Norbeck     | 75—58   |
| 2,595,292 | 6/1952  | Reece       | 75—122  |
| 3,356,489 | 12/1967 | Feichtinger | 75—46   |
| 2,871,008 | 1/1959  | Spire       | 75—59 X |
| 2,991,684 | 7/1961  | Wever       | 73—23 X |
| 3,459,537 | 8/1969  | Hornak      | 75—49   |
| 3,137,753 | 6/1964  | Feichtinger | 75—51 X |

|           |         |        |          |
|-----------|---------|--------|----------|
| 3,408,059 | 10/1968 | Hornak | 75—49 X  |
| 3,634,075 | 1/1972  | Hoff   | 75—129 X |

## FOREIGN PATENTS

|           |        |        |        |
|-----------|--------|--------|--------|
| 1,403,347 | 5/1965 | France | 164—57 |
|-----------|--------|--------|--------|

CHARLES N. LOVELL, Primary Examiner

J. E. LEGRU, Assistant Examiner

U.S. CL. X.R.

75—53, 59, 61